

Patented Aug. 3, 1926.

1,594,762

# UNITED STATES PATENT OFFICE.

MORRIS C. VAN GUNDY AND HOWARD DIMMIG, OF PORT ARTHUR, TEXAS, AS  
SIGNORS TO THE TEXAS COMPANY, OF NEW YORK, N. Y., A CORPORATION OF  
TEXAS.

## MANUFACTURE OF LUBRICANTS.

No Drawing.

Application filed October 13, 1921. Serial No. 507,551.

This invention relates to the production of normal lead oleate and the preparation of lubricating compounds therefrom.

In present methods of making lubricating compounds containing lead soap, it is customary to mix whale oil or other fish oil or oil containing a fatty acid with litharge or red lead while heating the ingredients to about 450° F. This results in the production of the basic lead oleate,



This basic salt is sticky and stringy in character, it is not permanently soluble in hydrocarbon oils, it does not reduce the viscosity of lubricating oil at low temperatures and is, in fact, wholly unsuited for use in the preparation of lubricating compounds.

When this basic salt is mixed with the lubricating oil considerable difficulty has been experienced in the past due to the fact that the insoluble bodies settle out.

Superior lubricating compounds may, however, be made by the use of the normal lead oleate,



since the normal salt is oily in character, is permanently soluble in oil and has the characteristic of reducing the viscosity at low temperatures of the lubricating stock with which it is compounded.

We have discovered that the normal lead oleate may be made by reacting oleic acid and lead oxid under certain critical conditions as to temperature.

In accordance with our invention any of the oxids of lead, preferably one of the lower oxids, and oleic acid in any suitable form, such as elaine or red oil, are mixed together and the temperature of the ingredients is raised to from about 500° F. to 525° F., the preferred temperatures being from 520° F. to 525° F. At a temperature of about 530° F., the normal lead oleate is decomposed and, therefore, temperatures in excess of 525° F. should not be used. Temperatures around 500° F. to 515° F. may be employed; however, the rate of reaction is so much reduced even at this slight reduction from the preferred temperature that such temperatures are not to be recommended and in practice we endeavor to hold the ingredients as near as may be between 520° F. to 525° F.

It is not practicable to have the materials entering into the reaction at the preferred temperature at the commencement of the operation since there would be considerable loss due to the volatilization of the elaine oil in case it were heated originally over 500° F. The result is that there are probably certain preliminary reactions occurring at the lower temperatures while the ingredients are being raised to the preferred temperature. It is very likely that the lead oxid and oleic acid react at the lower temperatures to form the basic lead oleate and steam and when a temperature of 520° F. to 525° F. is attained the basic salt is decomposed and the normal oleate formed, the reactions probably taking place about as follows:



During the heating, the ingredients are preferably agitated or stirred, the heating and agitation being continued until there is no free acid present and the resultant normal lead oleate is then allowed to cool somewhat, for example to about 200° F. after which it is mixed with lubricating oil to form the desired compound.

In lead soap lubricating compounds, such as car oils, for instance, made by prior methods of manufacture, a greater or less quantity of insoluble material is found to be contained in the compounds and these insoluble bodies readily settle out. These settling may be attributed to the use of the basic lead oleate and also to the presence of lead stearate and palmitate which are commonly found in car oils. These settling are not only insoluble in oil but moreover have no lubricating value. When preparing lubricating compounds in accordance with the present invention involving the use of the normal lead oleate, a homogeneous compound is formed with the lead soap completely in solution in the mixture and with no deposits or settling. The presence of the normal lead oleate adds to the lubricating value of the compound since the normal salt has an unctuous quality and is itself suitable for use as a lubricant.

The normal soap also possesses the property of reducing the viscosity at low tem-

peratures of the compound into which it enters below that of the oil stock with which it is mixed. The effect of the normal soap on paraffin oils is especially marked, the oleate apparently hindering in some manner the formation of wax crystals. The effect on asphalt base oils is in a less degree but the viscosity of the compound is also reduced at low temperatures below that of the oil stock. The practice of our invention is thus particularly adapted for the production of lubricants adapted for use at cold temperatures.

Various lubricating compounds may be prepared in accordance with our invention, such for example as car oils, driving journal compounds and other lubricants. The proportion of oleate used varies with the type of product desired. For example, summer car oils require less oleate than winter car oils. The proportion may vary from as low as 2%–10%, which is the proportion ordinarily used for car oils, for instance, to the higher proportions used in the preparation of greases.

Obviously many modifications and variations of the invention, as hereinbefore set forth, may be made without departing from the spirit and scope thereof, and therefore, only such limitations should be imposed as are indicated in the appended claims.

What we claim is:—

1. The process of manufacturing lubricants which comprises heating a mixture of oleic acid and lead oxid to approximately 520° F.–525° F. thereby forming normal lead oleate and then mixing said oleate with lubricating oil.

2. The process of manufacturing lubricants which comprises agitating a mixture of oleic acid and lead oxid maintained at approximately 520° F.–525° F. and then mixing the resulting product with lubricating oil.

3. The process of manufacturing lubricants which comprises gradually heating a mixture of oleic acid and lead oxid to approximately 520° F.–525° F., maintaining that temperature until no free acid is present and compounding the resulting product with lubricating oil.

4. The process of manufacturing lubricants which comprises gradually heating a mixture of oleic acid and lead oxid to approximately 520° F.–525° F., maintaining that temperature until no free acid is present, then permitting the mixture to cool to a relatively lower temperature and adding lubricating oil to form a lubricating composition.

5. The process of manufacturing lubricants which comprises heating a mixture of oleic acid and lead oxid to a temperature of at least 500° F. but not in excess of 530° F. and compounding the product formed with hydrocarbon oil.

6. The process of manufacturing lubricants which comprises heating a mixture of oleic acid and lead oxid to a temperature sufficiently high to produce a reaction resulting in normal lead oleate, but not in excess of 530° F. and thereafter mixing the said oleate with lubricating oil.

In witness whereof we have hereunto set our hands this 3rd day of October, 1921.

MORRIS C. VAN GUNDY.  
HOWARD DIMMIG.